

## UNITED STATES PATENT OFFICE

2,604,452

## TWISTER RING LUBRICANT

Arnold J. Morway, Clark Township, Union County, and David W. Young, Roselle, N. J., assignors to Standard Oil Development Company, a corporation of Delaware

No Drawing. Application December 30, 1950,  
Serial No. 203,794

6 Claims. (Cl. 252—51.5)

1

This invention relates to a lubricating grease composition having characteristics that make it especially desirable as a twister ring lubricant. More particularly, this invention relates to a twister ring grease prepared by thickening a white petrolatum to a grease consistency with an N-acyl amino phenol.

In the art of textile manufacture, a lubricating problem exists which causes a great deal of lost time, that of twister ring lubrication. In the textile manufacturing step in which this problem exists, the untwisted yarn is twisted and wound at high speeds upon spools in preparation for the weaving looms. In the twisting and winding operation two or more yarns, or plies, are brought together and twisted into a single strand and then wound on the spool, or bobbin, which is mounted on a spindle within a twister frame. The bobbin stands vertically within a circular metal ring called a twister ring mounted on the twister frame. Riding upon the twister ring and travelling freely on its circumference is the traveler, a looped metal member made of steel or bronze. In the process of twisting and winding, two or more yarns or plies pass through the loop of the traveler are twisted by its rotational movement around the twister ring, and are wound on the bobbin, rotating upon the spindle. The bobbin rotates at speeds in the neighborhood of 7,000 R. P. M. or more and the traveler moves around the twister ring at speeds almost as great. The extremity of the need for lubricating of the twister ring is emphasized when one considers that the traveler, weighing only a fraction of an ounce, may develop several pounds of centrifugal force at top speeds.

Twister ring greases have hitherto been prepared using as a base a white oil and as thickening agents a mixture of calcium and sodium soaps. These greases have met with considerable success but are not perfectly satisfactory in all instances since careful control is necessary in their manufacture to obtain the exact degree of viscosity necessary for satisfactory lubrication. If the grease is too viscous, it will be thrown from the ring, discoloring the yarn, and resulting in a failure of lubrication causing high traveler wear and high yarn tensions which increases the breakage rate. A grease that is too thin will drip and spatter, with identical results.

It has now been found that excellent twister ring greases may be prepared by thickening a white petrolatum with an N-acyl amino phenol containing from 14 to 22 carbon atoms in the acyl portion thereof. These novel greases have

2

the advantage of not modifying the texture of the petrolatum greatly while more than doubling its melting point. In addition, the amino phenol imparts oxidation resistance characteristics and prevents darkening of the petrolatum. This prevents yarn discoloration and the formation of unpleasant odors in the spinning room.

In general, the greases of invention are prepared simply by heating the desired petrolatum with from 1.0% to 10.0%, preferably 3% to 6%, by weight of a desired N-acyl amino phenol to a temperature of the melting point of the phenol, usually 240° to 275° F. When the N-acyl amino phenol is completely in solution the mass is cooled without agitation and upon solidification, the product is a smooth unctuous material of excellent appearance.

The petrolatum used in the formulation of the greases of invention may be any of the white petrolatums having melting points within the range of from 75° to 125° F. and ASTM consistencies of from 200 to 325 mm./10. The preferred embodiment of the invention contemplates, however, the use of a white petrolatum having a melting point within a range of from 112° to 124° F. with an ASTM consistency of from 240 to 290 mm./10. If petrolatums of greater consistencies are employed, it may be necessary to blend with them a minor amount of a white oil to obtain desired handling properties.

The N-acyl amino phenol used for the preparation of the greases of invention have the general formula:



40 whereon R is an alkyl group containing from 14 to 22 carbon atoms, preferably an alkyl group non-benzenoid in nature, and whereon R' and R'' are hydrogen atoms or alkyl groups containing from 1 to 20 carbon atoms.

45 The preferred embodiment of this invention contemplates the use of compounds according to the formula above whereon R' and R'' are hydrogen atoms, and whereon R is a straight chain aliphatic group containing from 16 to 20 carbon atoms, that is, the N-acyl p-amino phenols. Exemplary of these preferred compounds are N-palmitoyl p-amino phenol, N-stearoyl p-amino phenol, and N-arachidoyl p-amino phenol, with N-stearoyl p-amino phenol being especially preferred.

The alkylated N-acyl p-amino phenols exemplified by the formula above when R' and R'' are alkyl groups containing from 1 to 20, preferably 4 to 15, carbon atoms are also operable in this invention. Compounds such as N-n-valeryl-4-amino-3-pentadecyl phenol, N-n-propanoyl-4-amino-3-pentadecyl phenol, N-n-pentanoyl-4-amino-2,6-di-tert.-butyl phenol, N-n-hexyl-4-amino-2-hexyl phenol are examples of the alkylated phenols operable.

If desired the amino phenols having the amino group meta to the hydroxy group may be used in practicing this invention. That is the N-acyl m-amino phenols, either alkylated or not, may be used as petrolatum thickeners.

The preparation of these N-acyl amino phenols is accomplished by simply admixing the desired acid or acid chloride with the desired amino phenol and heating the mixture under proper reaction conditions. The reaction proceeds smoothly splitting off water or hydrogen chloride, giving the desired amino phenol as an end product. It may then be purified by any of the methods known to the art.

The method for the preparation of an operable p-amino phenol is typified by the following:

One mol of p-amino phenol was placed in a glass round bottomed flask fitted with a reflux condenser with an azeotropic take off arm. There was added to the flask one mol of stearic acid and about 50 gm. of xylene. The xylene served as an entraining agent for the water formed during the course of the reaction. The flask was then heated to the xylene reflux temperature and kept at that temperature for about 5 hours, or until the theoretical water (1 mol) had been removed. The contents of the flask was then emptied into an evaporating dish and heated on a steam bath until the last trace of xylene was removed. The product was then recrystallized from acetic acid and there resulted a colorless N-stearoyl p-amino phenol (melting point 132° C.).

The following examples are given to more explicitly point out this invention, it being kept in mind that they are exemplary only and do not restrict in any way the inventive concept as set out above.

#### EXAMPLE I

To 98% by weight of a white petrolatum having a melting point of 110° F. and an ASTM penetration of 275 mm./10 there was added 2.0% by weight of N-stearoyl p-amino phenol, prepared by reacting with p-amino phenol a commercial stearic acid derived from tallow and containing palmitic acid. The temperature of the mixture was then raised with agitation to the melting point of the amino phenol, about 240° F. The mixture was then allowed to cool to room temperature without agitation, and there resulted a smooth unctuous grease composition of generally excellent appearance. The dropping point of this grease composition was 220° F. and the ASTM penetration 275 mm./10.

#### EXAMPLE II

It has been found that N-stearoyl p-amino phenol has excellent thickening properties, but little anti-oxidant effect, while conversely, the N-lauroyl p-amino phenol has little thickening ability but imparts excellent resistance to oxidation to these grease compositions. In order to utilize these properties, twister ring lubricants were prepared in accordance with the procedure detailed in Example I above employing mixtures

of the N-stearoyl and N-lauroyl p-amino phenols dispersed in a white petrolatum having a dropping point of 106° F. and an ASTM penetration of 275 mm./10. These grease compositions, in addition to the standard ASTM dropping point determinations, were subjected to the Norma-Hoffman bomb test to determine their resistance to oxidation. In this test, a sample of the grease was placed in a stainless steel bomb and oxygen was admitted until the pressure stabilized at 110 p. s. i. The test data is reported in hours to a 5-pound pressure drop, the pressure drop being due to the oxidation of the sample. Test data is reported in Table I, below:

Table I  
TWISTER RING GREASES

| Thickener                       | Dropping Point °F | ASTM Penetration mm./10 | N-H Test Hrs. to 5 p. s. i. Drop |
|---------------------------------|-------------------|-------------------------|----------------------------------|
| Petrolatum                      | 106               | 275                     | (1)                              |
| 2.0% N-stearoyl p-amino phenol  | 240               | 275                     | 70                               |
| 1.75% N-stearoyl p-amino phenol | 232               | 275                     | 400+                             |
| .25% N-lauroyl p-amino phenol   | 222               | 275                     | 400+                             |
| 1.5% N-stearoyl p-amino phenol  | 208               | 275                     | 400+                             |
| 1.0% N-stearoyl p-amino phenol  | 200               | 275                     | 400+                             |
| 2.0% N-lauroyl p-amino phenol   | 200               | 275                     | 400+                             |

<sup>1</sup> 30 p. s. i. in 70 hrs.

If it is desired to make a higher melting product, a minor amount of a common grease making soap may be incorporated in the greases of invention. For instance, alkali metal or alkaline earth metal soaps of any of the commonly known fatty acids may be used. A lubricant containing 2.0% N-acyl p-amino phenol and 6.0% lithium stearate dispersed in the petrolatum will have the consistency of a grease containing 21.0% or more of the soap. This results in an obvious economic advantage in the preparation of these lubricants. In addition in cases where a white oil is employed in combination with the petrolatum to modify and give the desired consistency, the N-acyl p-amino phenol, whether employed as the thickener alone or in combination with metal soap thickeners, prevents, to a large degree, exuding of the oil in service or in storage.

To summarize briefly, this invention relates to improved twister ring lubricants consisting of a white petrolatum, alone or in combination with a white oil, thickened to a grease consistency with an N-acyl p-amino phenol. These greases have desirable uniform consistencies and excellent anti-oxidant characteristics.

What is claimed is:

1. A new and improved twister ring lubricant consisting essentially of a white petrolatum containing dispersed therein from 1% to 10% by weight, based on the weight of the total composition, of an N-acyl p-amino phenol, the acyl group of which contains from 12 to 22 carbon atoms.

2. A new and improved twister ring lubricant consisting essentially of a white petrolatum containing dispersed therein from 1% to 10% by weight, based on the weight of the total composition, of an N-acyl p-amino phenol, the acyl group of which contains 16 to 20 carbon atoms.

3. A new and improved twister ring lubricant consisting essentially of a white petrolatum containing dispersed therein from 3 to 6% by weight, based on the weight of the total composition, of an N-acyl p-amino phenol, the acyl group of which contains from 16 to 20 carbon atoms.

4. A new and improved twister ring lubricant consisting essentially of a white petrolatum having a melting point within a range of from 75° to 120° F., containing dispersed therein from 3 to 6% by weight, based on the weight of the total composition, of an N-acyl p-amino phenol, the acyl group of which contains from 16 to 20 atoms per molecule.

5. A new and improved twister ring lubricant consisting essentially of a white petrolatum having a melting point within a range of from 112 to 124° F., containing dispersed therein from 3 to 6% by weight, based on the weight of the total composition, of N-stearoyl p-amino phenol.

6. A new and improved twister ring lubricant consisting essentially of a white petrolatum con-

taining dispersed therein from 1 to 10% by weight, based on the weight of the total composition, of a mixture of at least two N-acyl p-amino phenols, the acyl groups of which correspond to the acid radicals of stearic and lauric acid.

ARNOLD J. MORWAY.  
DAVID W. YOUNG.

## REFERENCES CITED

The following references are of record in the file of this patent:

## UNITED STATES PATENTS

| 15 | Number    | Name     | Date          |
|----|-----------|----------|---------------|
|    | 2,065,857 | Hilliker | Dec. 29, 1936 |